

Dec. 15, 1931.

R. C. BENNER ET AL  
OPERATION OF SILICON CARBIDE RESISTORS IN  
PROTECTIVE ATMOSPHERES  
Filed July 30, 1930

1,837,179

2 Sheets-Sheet 1

Fig. 1.



Fig. 2.



INVENTORS  
RAYMOND C. BENNER  
GEORGE J. EASTER  
CLARENCE E. HAWKE  
BY

Thomas C. MacKay  
ATTORNEY

Dec. 15, 1931.

R. C. BENNER ET AL

1,837,179

OPERATION OF SILICON CARBIDE RESISTORS IN  
PROTECTIVE ATMOSPHERES

Filed July 30, 1930

2 Sheets-Sheet 2

Fig. 3.



BY

INVENTORS  
RAYMOND C. BENNER  
GEORGE J. EASTER  
CLARENCE E. HAWKE

Thomas C. Mackay  
ATTORNEY

## UNITED STATES PATENT OFFICE

RAYMOND C. BENNER AND GEORGE J. EASTER, OF NIAGARA FALLS, NEW YORK, AND CLARENCE E. HAWKE, OF METUCHEN, NEW JERSEY, ASSIGNEES TO THE CARBORUNDUM COMPANY, OF NIAGARA FALLS, NEW YORK, A CORPORATION OF PENNSYLVANIA

## OPERATION OF SILICON CARBIDE RESISTORS IN PROTECTIVE ATMOSPHERES

Application filed July 30, 1930, Serial No. 471,714, and in Canada March 20, 1929.

This invention relates to the prolongation of the useful life of silicon carbide resistors, and to a method of operating such resistors whereby high temperatures can be maintained over prolonged periods of time without causing undesirable changes in electrical properties. The present application is a continuation in part of our co-pending application, United States Serial No. 324,416, filed December 7, 1928.

The use of silicon carbide heating elements of a rigid or self-sustaining character in electric furnaces is well known. These resistors offer a number of advantages over the other types of elements in common use. They are suitable for operation at temperatures considerably in excess of that possible with a metal resistor such as "nichrome". The resistor material has a much higher specific resistance than graphite, so that elements having a fairly large surface for the dissipation of heat can be operated on the standard line voltages, without the use of low voltage transformers.

Silicon carbide resistors are of such a character that they have always been regarded as stable in air. In contrast with graphite resistors, which are subject to burning and rapid mechanical disintegration when operated in air at temperatures above a dull red heat, a silicon carbide resistor can be operated continuously in the open air at temperatures up to 1300° C. for more than 1000 hours without any visible change, except for possibly a slight change in color. The silicon carbide resistor is practically the only element which can be operated in air above 1100° C., since graphite, tungsten, molybdenum and other commercial materials of high melting point all oxidize so rapidly that their operation at high temperatures without protection is impossible. In the case of graphite, the material actually burns and is reduced to ash unless protected from oxidation, so that the necessity of protection is evident. However, silicon carbide resistors have been regarded as being of a different type from the easily oxidizable heating elements, and because of their comparative stability they have always

been operated without protection since their first introduction into commercial use.

Although silicon carbide resistors possess many advantages, there are certain undesired changes in electrical properties which take place during the life of the element as ordinarily operated. The electrical resistance does not remain constant during use, but is continually changing throughout the life of the resistor. This change takes place even when the element is operated at fairly low temperatures, as for example 700-800° C., although the element is physically and mechanically stable at much higher temperatures. The increase in resistance during the first few hours of operation is often appreciable, and after 1000 hours the increase may be as much as 50 to 100 per cent. In order to counteract the changing resistance it is necessary to continually alter the voltage across the terminals of the resistor if a constant power input is to be maintained.

The temperature coefficient of resistance also changes during the life of the element, the coefficient becoming considerably more negative as the element increases in electrical resistance. This factor is of considerable importance in the operation of an electric furnace, since a strongly negative temperature coefficient makes the regulation of the power input and the maintenance of a constant temperature very difficult. In operating the element at a definite voltage, any increase in temperature will cause an increase in current, and the increased current will cause a still further increase in temperature, these increases being cumulative in their effect. In a very few minutes both the resistor and the contents of the furnace can be damaged or completely destroyed by what was originally only a slight temperature fluctuation.

Although the difficulty of variable rather than constant electrical properties has always been considered as inherent in the operation of this type of resistor, we have found that the electrical properties of a silicon carbide element can be kept practically constant over prolonged periods of time by operating the resistor in a non-oxidizing atmosphere. In

our improved method of operation, both the original resistance of the element and the original temperature coefficient of resistance are preserved by operation under non-oxidizing conditions. In addition, the useful life 5 of the resistor is greatly prolonged over that which has heretofore been regarded as satisfactory for a resistor of this type. The factor limiting the useful life of a silicon carbide heating element has always been that of increased electrical resistance and change of 10 resistance-temperature characteristics rather than physical or mechanical disintegration. In the past it has been customary to operate 15 the resistor without protection until the electrical resistance increased from 50 to 100 per cent, whereupon the element was considered unfit for further use and was discarded.

Recent developments in connection with 20 the manufacture of silicon carbide resistors have made possible the production of an element in which the temperature coefficient of resistance is positive within the operating range. In several co-pending applications 25 (U. S. Serial No. 324,418, filed December 7, 1928; U. S. Serial No. 324,419, filed December 7, 1928; and U. S. Serial No. 485,998, filed October 2, 1930) we have disclosed methods 30 of utilizing this property to maintain a practically constant temperature within an electric furnace. The electrical resistance of this type of element increases as the temperature is increased from approximately 800° C. to 1500° C., and as the furnace becomes over-heated, the power input at a given voltage is 35 considerably decreased. On the other hand, if the interior of the furnace is cooled by the introduction of a cold charge, the power input is increased until the furnace returns to 40 normal temperature. A degree of regulation is afforded which often amounts to from 30 to 40 per cent of the power input.

When the resistors are operated in the usual manner in air, the positive temperature 45 coefficient is not retained with prolonged use. The increase in resistance with rising temperature becomes less as the element is used, until the regulation of the power input by this means is reduced to the point where it is of 50 little practical value. After the element has increased considerably in resistance, the effect due to the positive temperature coefficient is often completely lost, and the temperature coefficient may even become negative 55 throughout the entire range of operating temperatures, thus causing a reverse effect from that desired.

Our method of operation in which a protective atmosphere is used affords a means of 60 preserving the original positive temperature coefficient of resistance of the element, and thus makes available the regulation of both power input and temperature throughout the useful life of the resistor.

65 We believe that the maintenance of con-

stant electrical properties by operation in a non-oxidizing atmosphere may be explained as being due to the prevention of the small amount of oxidation which normally takes place during the operation of the element in 70 air. Although the actual amount of oxidation is small from a physical or mechanical standpoint, it is apparently sufficient to cause a fairly rapid deterioration in electrical properties. The resistors are composed of 75 an aggregation of small silicon carbide grains, and since the element is quite porous and the grains are not in intimate contact over their entire surface area, a considerable portion of the electrical resistance arises from 80 these surfaces of intergranular contact. Even a slight amount of oxidation, if it causes an insulating film to form at the points or areas of intergranular contact, will have a 85 marked effect on electrical properties. Resistors have been observed in which the electrical resistance had increased appreciably, but the actual amount of oxidation was so 90 small that the surface of the silicon carbide crystals possessed an iridescent appearance 95 characteristic of thin interference films. As is well known, an oxide film capable of producing interference phenomena has a thickness of the order of magnitude of the wavelengths of visible light.

By the use of a protecting atmosphere, a silicon carbide resistor can also be operated at a considerably higher temperature than has heretofore been possible with this type of 100 element without affecting the electrical properties. The upper temperature limit for a silicon carbide resistor has previously been regarded as being approximately 1400-1500° C., and even at this temperature the increase in resistance and change in temperature coefficient of resistance is very rapid 105 when the element is operated in air.

In the operation of resistors composed of silicon carbide, they have occasionally been 110 found to warp or bend, even when no appreciable softening of the resistor material takes place. In the operation of resistors in a non-oxidizing atmosphere, this phenomenon has not been observed. It seems probable that the warping is due to differential expansion 115 caused by localized oxidation. It is known that silicon carbide refractories often expand when exposed to oxidizing conditions.

For the protection of the resistors, any gas 120 which will not react with silicon carbide at the temperature of operation of the element may be used. We prefer to use carbon monoxide or an atmosphere containing an appreciable proportion thereof, although nitrogen or other gases having less reactivity than ordinary air may be used. If desired, the resistor may be embedded in a solid protecting material, as for example carbon in the form of lamp black or powdered coke. If an 125 inert gas rather than a solid embedding 130

material is used, the elements may be placed directly within the heating chamber.

A reducing atmosphere containing a considerable proportion of carbon monoxide can be formed by introducing carbon, preferably in finely divided form, into the heating chamber. The amount of carbon necessary to remove the oxygen from a cubic foot of air at 1100° C. is comparatively small, being approximately 2.5 grams or .005 pound, although it is of course desirable to have a considerable excess over the theoretical amount required. Both coke and charcoal have a considerable amount of ash, so that it is desirable to use purer forms of carbon such as lamp black or petroleum coke for the removal of the oxygen from the interior of the muffle. A thin layer of lamp black on the floor of the muffle will remain for several days without being consumed, if reasonable precautions are taken not to expose the heating chamber to the open air.

A preferred method of carrying out our invention is illustrated in the accompanying drawings, in which:

Figure 1 is a vertical section of a form of furnace in which the muffle is subjected to a non-oxidizing atmosphere, the resistors being directly in the muffle;

Figure 2 is a vertical section of a modified furnace in which reducing gas is introduced directly into the heating chamber; and

Figure 3 is a vertical section through the center of the furnace, taken on the line 3—3 of Figure 2.

Referring to the drawings in more detail, the resistors 2, which are composed principally of silicon carbide, are mounted in the usual manner, using either self-cooled or water-cooled terminals. In order to secure uniform heat distribution around and beneath the charge, the upper portion of which is exposed to direct radiation, it is desirable that the lining 4 be composed of highly conductive refractory, as for example, one having a thermal conductivity in excess of .006 calorie/cm<sup>2</sup>/sec/° C., as disclosed in our pending application, U. S. Serial No. 324,419, filed December 7, 1928. Silicon carbide or fused alumina are examples of such refractories.

The success obtained in maintaining a non-oxidizing atmosphere within the muffle will depend upon the degree to which the infiltration of air is prevented. For this reason, it is desirable to use a dense or comparatively impermeable refractory, or else a porous refractory surrounded by granular or powdered carbon or other carbonaceous material.

In the form of furnace shown in Figure 1, the resistors 2 are placed adjacent to a porous wall 3 of highly conducting refractory such as recrystallized silicon carbide, which conducts heat to granular carbon within the wall of the furnace. The carbon

is also shown as extending down through the side walls of the furnace, where it is separated from the interior by the wall 4 of similar material to that composing the wall 3. The silicon carbide is an excellent conductor of heat, so that the outer portion of the wall may be operated at incandescence, and any air filtering into the muffle, through the porous walls will first come in contact with the hot carbon and the oxygen will be removed therefrom to form carbon monoxide. The granular or powdered carbon will afford effective thermal insulation between the inner and outer walls of the furnace. Fresh carbon may be added through an opening 80 which is ordinarily closed by the plug 6, or through the openings 7. If desired, a small quantity of finely divided carbon may be placed within the heating chamber.

Figures 2 and 3 show the direct use of a non-reacting gas independent of granular carbon to afford protection for the resistors. Producer gas or other suitable gas is introduced into the muffle through conduits 11, which are preferably located near the ports 90 where the resistor terminals penetrate the furnace wall. The flow of gas may be controlled by means of valves 12.

In the furnaces described above, in which the resistors are placed within the heating chamber, the non-oxidizing atmosphere serves to protect both the resistors and the furnace charge. This factor is particularly important in the case of heat-treating work, where the metal must be protected from scaling. There are many other instances where it is important to protect the ware itself as well as the resistors.

The means which we have described for carrying out our invention may of course be varied according to the design and type of furnace in which the resistors are employed. Our invention may be defined as being within the scope of the following claims.

1. In an electric furnace, a chamber for ware to be treated, silicon carbide resistors within said chamber, the walls of said chamber being composed of refractory which is permeable to gases, and a granular carbon packing around said chamber walls.

2. In an electric furnace, a chamber for ware to be treated, silicon carbide resistors within said chamber, the walls of said chamber being composed of refractory which is permeable to gases and possesses a high thermal conductivity, and a granular carbon packing around said chamber walls.

3. The method of operating a silicon carbide resistor which comprises surrounding the resistor with a non-oxidizing atmosphere.

4. The method of operating a silicon carbide resistor which comprises surrounding the resistor with an atmosphere having a substantial proportion of carbon monoxide.

5. An electric furnace comprising in com-

bination a resistor consisting mainly of silicon carbide, an enclosing muffle wall about the resistor, and means for supplying a non-oxidizing atmosphere around said resistor and about ware under treatment in the muffle.

6. In an electrical resistance furnace a silicon carbide resistor, an adjacent muffle whose walls are composed of silicon carbide, and means for maintaining a non-oxidizing atmosphere around the resistor and muffle.

In testimony whereof we affix our signatures.

RAYMOND C. BENNER.

GEORGE J. EASTER.

CLARENCE E. HAWKE.